

Jan. 15, 1935.

E. G. HERBERT

1,988,040

PROCESS FOR THE TREATMENT OF METALS

Filed June 9, 1932



Fig. 1.



Fig. 4.



Fig. 2.



Fig. 5.



Fig. 3.



Fig. 6.

Inventor:

Edward G. Herbert

By his Attorney: Walter Gunow

## UNITED STATES PATENT OFFICE

1,988,040

## PROCESS FOR THE TREATMENT OF METALS

Edward Geisler Herbert, West Didsbury,  
Manchester, EnglandApplication June 9, 1932, Serial No. 616,175  
In Great Britain June 22, 1931

8 Claims. (Cl. 148—10)

This invention refers to a new or improved process for the secondary treatment of metals and other substances in which fluctuations in their physical properties, such as hardness or ductility, occur after a primary thermal, mechanical, or magnetic treatment.

It has been discovered that metals which have undergone certain thermal or mechanical treatments exhibit a series of periodic changes of hardness during a period of ageing immediately following the treatment, the hardness changes being associated with changes of other physical properties such as ductility. The fluctuations of hardness consist of alternate increases and decreases, the periodicity of the fluctuations generally tending to increase, so that the first change, which may be either an increase or a decrease of hardness, may occupy only a few minutes, and later changes will usually occupy many hours.

In some cases the first change occupies three or four hours or longer, and subsequent changes generally occupy longer periods. It is believed that this phenomenon is not peculiar to metals, but that it takes place in some other crystalline substances.

The treatment which gives rise to these fluctuations may be thermal, such as quenching from a high temperature, or heating, or annealing, or it may be mechanical such as rolling or hammering, or bombardment with steel balls.

It has been discovered further that the changes of hardness of a metal set up by the magnetic treatment, (generally consisting of rotation in a magnetic field) described in my application of prior date No. 474,309, filed 9th August, 1930, are also periodic fluctuations. It is believed that the periodic fluctuations set up by thermal, mechanical and magnetic treatments are essentially similar in character, and the hypothesis has been advanced that they are due to precession in the systems of electrons giving rise to fluctuations in molecular cohesion.

When the hardness fluctuations damp out they generally leave the metal with physical properties different from those which it possessed immediately after the treatment (thermal, mechanical or magnetic) which gave rise to the fluctuations. Thus, steel which has been quenched from a high temperature, or annealed at a low temperature after having been work hardened, or which has been hardened by cold working or magnetically treated according to my said patent application No. 474,309, usually reaches stability in a condition of hardness considerably higher than that which it possessed immediately after

the application of the treatment, but its final hardness is usually less than the maximum and greater than the minimum which it has passed through in the course of its fluctuations during the period of ageing which intervenes between the original treatment and the condition of stability.

It is now found that as regards their immediate and/or ultimate physical properties, the substances subject to the aforesaid fluctuations of physical properties respond to a further or secondary magnetic treatment differently at different stages of their aforesaid fluctuations.

The object of this invention is to take advantage of such discovery as regards the effect of the further or secondary treatment, to accentuate or decrease one or more of the physical properties of the substance beyond the limits otherwise obtainable, in order to obtain an optimum state of hardness for the particular purpose in hand.

The present invention consists in applying to the substance at a selected phase of its fluctuations a secondary magnetic treatment, such as will stabilize the metal in the condition it has then reached, or will influence the subsequent fluctuations in such a manner as may be desired.

In cases where the fluctuations resulting from the primary treatment of metal have damped out, the invention also consists in first reinstating them by a primary treatment consisting in rotating the metal in a strong magnetic field and then applying the secondary treatment at the selected phase.

The terms "primary treatment" and "secondary treatment" are used in a relative sense, the primary treatment being that which causes the fluctuations of hardness, and the secondary treatment that which stabilizes them.

The secondary treatment may consist of the application of a stationary magnetic field, or a rotating magnetic field, or a de-magnetizing process as hereinafter explained, and it may be applied either to magnetic or non-magnetic metals, at any selected phase of fluctuations set up by previous thermal, mechanical, or magnetic disturbance, according to the result desired. While an important practical application of the secondary treatment is that of improving the physical properties of hard steel used in cutting tools and other structures and of improving the physical characteristics of unhardened steels used for mechanical structures, it is to be particularly noted that both the primary and secondary magnetic treatments have been found effective when applied to non-magnetic metals, such as brass, and

that known by the registered Trade Mark Duralumin, and may be applied also to non-metallic bodies whose electronic systems are susceptible to the influence of magnetic fields.

5 An example of the carrying out of the invention is in the treatment of a steel wire which has been treated by rotating it in a magnetic field according to my patent application No. 474,309, and which after such treatment would normally 10 pass through a series of hardness fluctuations characterized by a maximum hardness immediately after treatment, a minimum  $\frac{1}{2}$  hour after, a maximum  $1\frac{1}{2}$  hours after, a minimum 5 hours after, and a maximum 12 hours after the 15 magnetic treatment. Instead of permitting this normal course of fluctuations, I select a particular phase such as the  $1\frac{1}{2}$  hour maximum, or the 5 hour minimum, and at that particular period of the ageing process I subject the steel to a 20 secondary treatment by placing it in a constant magnetic field for several minutes, or as long as may be found effective, or by a de-magnetizing process, the result of this treatment being to stabilize the metal in the physical condition which 25 it has attained when the secondary treatment is applied.

Another example of the carrying out of the invention is in the treatment of a steel which has been hardened by quenching and which normally 30 would pass through fluctuations of hardness such that the hardness reaches a maximum 3 hours after quenching and a minimum 7 hours after quenching. Instead of permitting this course of fluctuations, I select a particular phase such as 35 the 3 hour maximum and at that phase subject the steel to a secondary treatment by placing it in a constant and stationary magnetic field for a period of, say 2 minutes. The effect of this is found to be either a stabilization of the steel in 40 the condition of maximum hardness which it had attained when the secondary treatment was applied, or, more frequently, to cause an immediate further increase of hardness and some fluctuations of hardness which eventually damp 45 out leaving the metal in a stable condition characterized by greater hardness than it possessed when the secondary treatment was applied.

The diagrams shown in the accompanying drawing represent the hardness time curves of 50 specimens referred to in the following examples of carrying out the invention.

A razor blade was treated primarily by rotation in a magnetic field with the result that the hardness fell immediately and then rose considerably, 55 ultimately (after 20 hours) falling to its original level. Fig. 1 is a graph of the test.

Another razor blade was similarly treated, but at the end of two hours a secondary magnetic treatment was applied to the blade by placing it 60 in a stationary magnetic field for 5 minutes. The result was an immediate rise in hardness, and a further progressive rise during 25 hours, the final hardness being much higher than the previous maximum. Fig. 2 illustrates the changes of hardness.

Further consideration of the effects produced by the secondary treatment in a constant magnetic field, and especially of the fact that in some cases the constant field does not immediately 70 stabilize but sets up new fluctuations of a somewhat violent character and of shorter time periodicity than those which are normally taking place, has suggested that the most appropriate secondary treatment for stabilization would be 75 not in a constant magnetic field but by a de-

magnetizing process. This would usually consist in rotating the substance in a strong magnetic field and gradually withdrawing it from the influence of the field or alternatively, rotating the substance in a strong magnetic field, and gradually weakening the field to zero, or as a further alternative, simultaneously reversing and weakening the field, the effect in each case being to set up changes of polarity of gradually decreasing intensity so as finally to leave the substance magnetically neutral. Other demagnetizing processes such as an alternating magnetic field may be employed. Where the secondary treatment results in new fluctuations, a second stabilizing treatment may be given at a selected 15 phase of such new fluctuations.

Fig. 3 illustrates the hardness changes in a razor blade treated as in the previous examples, except that the secondary treatment was for 1 minute only, and subjected to a second stabilizing 20 treatment after passing the induced maximum.

Fig. 4 illustrates the comparative hardness of two pieces of steel wire, each treated in a magnetic field (by being given one turn in forty seconds) and one allowed to age normally as 25 shown by the dotted graph, and the other stabilized by a secondary magnetic treatment for one minute and demagnetized, as shown by the full line graph.

The secondary treatment sometimes results in 30 an immediate decrease in hardness, followed by a rise to a maximum higher than that which preceded the secondary treatment. Fig. 5 illustrates such a change which took place in a specimen of Cobalt high speed steel stabilized by treatment 35 for 3 minutes in a stationary field.

Similarly, if a phase of minimum hardness is selected for the secondary treatment, the metal being placed in the constant magnetic field at that phase of its fluctuations, the effect will 40 usually be an immediate decrease of hardness below the selected minimum, and certain fluctuations which eventually damp out leaving the metal less hard than when the secondary treatment was applied. See the graph in Fig. 6.

It will be understood that a change of hardness is always associated with changes in other physical properties such as ductility, and the purpose of the secondary treatment will often be to induce some useful physical property in the metal, 50 of which the hardness change is merely a symptom.

Brass has been stabilized by treatment in a field of 23,000 gauss strength.

In the case of the secondary magnetic treatment, it may be carried out by apparatus consisting of a two-part table connected with and forming extensions of the poles of the magnet. The parts of the table are adjustable and reversible and are each shaped so that different 60 strengths and distributions of the magnetic field are thereby obtainable, the substance to be treated being placed across the gap between the two parts of the table. Further, the magnet will preferably be designed so as to provide either a 65 rotating magnetic field, or a constant magnetic field or a de-magnetizing field.

What I claim is:—

1. The process of producing an optimum state of hardness in metals, which consists in subjecting the metals to a primary treatment to produce periodic increase and decrease of hardness, in observing by means of a hardness testing instrument the fluctuations of hardness following such treatment, in selecting a phase of fluctua- 75

tion for a secondary treatment, the selection being governed by the relationship of the desired optimum hardness to the initial hardness set up by the primary treatment, and in applying a 5 secondary treatment at such selected phase by placing the metals in a locally generated magnetic field to stabilize the fluctuations.

2. The process claimed in claim 1 wherein the secondary treatment is effected by placing the 10 metal in the locally generated magnetic field at a selected maximum phase of hardness fluctuation, to produce a stabilized ultimate condition of hardness higher than that immediately preceding the secondary treatment.

15 3. The process claimed in claim 1, wherein the secondary treatment is effected by placing the metal in the locally generated magnetic field at a selected minimum phase of hardness fluctuation to produce a stabilized ultimate condition of 20 hardness lower than that immediately preceding the secondary treatment.

4. The process of producing an optimum state 25 of hardness in metals, which consists in subjecting the metals to a primary hardening treatment, in observing by means of a hardness testing instrument the fluctuations of hardness following such treatment, in selecting a particular phase of fluctuation for a secondary treatment and in applying a secondary treatment at such selected 30 phase by placing the metals in a locally generated constant magnetic field to stabilize the fluctuations.

5. The process of producing an optimum state of hardness in ferrous metals, which consists in

subjecting the metals to a primary hardening treatment, in observing by means of a hardness testing instrument the fluctuations of hardness following such treatment, in selecting a particular phase of fluctuation for a secondary treatment and in applying a secondary treatment at such selected phase by placing the metals in a locally generated constant rotating magnetic field to stabilize the fluctuations.

6. The process of producing an optimum state 10 of hardness in ferrous metals, which consists in subjecting the metals to a primary hardening treatment, in observing by means of a hardness testing instrument the fluctuations of hardness following such treatment, in selecting a particular 15 phase of fluctuation for a secondary treatment and in applying a secondary treatment at such selected phase by subjecting the metals to the demagnetizing influence of a locally generated variable magnetic field to stabilize the fluctuations.

7. The process claimed in claim 1 characterized by the further steps of observing fluctuations set up by the secondary treatment, selecting a particular phase of such new fluctuations and 25 applying a second stabilizing treatment by again placing the metal within a locally generated magnetic field.

8. The process claimed in claim 1 wherein the primary treatment consists in placing the metal 30 within a locally generated magnetic field to produce fluctuations of hardness.

EDWARD GEISLER HERBERT.